

## UNITED STATES PATENT OFFICE

2,603,656

## PHOTOGRAPHIC DEVELOPING AGENTS.

Elmore Louis Martin, Wilmington, Del., assignor  
to E. I. du Pont de Nemours and Company,  
Wilmington, Del., a corporation of Delaware

No Drawing. Application February 27, 1951,  
Serial No. 213,051

4 Claims. (Cl. 260—509)

1

This invention pertains to a new class of N-substituted aminoaniline derivatives. More particularly it pertains to N-alkyl-N-(sulfophenoxy)alkylanilines. These compounds are useful as photographic developing agents.

Various arylendiamines have been used as photographic developing agents, but the most important of them, namely, para-phenylenediamine and its lower N,N-dialkyl derivatives have the disadvantage that they are readily absorbed by the skin and give rise to dermatitis. Since these agents are strong photographic developers and readily couple with color formers during the development of latent silver halide images to produce quinoneimine or azomethine dye images in situ with the silver images, they are used in most commercial processes of color photography. The compounds, however, due to their toxicity constitute a health hazard in photographic developing laboratories.

An object of this invention is to provide a new class of photographic developing agents. A further object is to provide a new class of photographic developing agents which are useful in chromogenic development and are free from toxic effects. The more specific object is to provide a new class of N-alkyl-N-(sulfophenoxy)alkylanilines. Still other objects will be apparent from the following description of the invention.

The new compounds of this invention may be represented by the following general formula:



where R is a hydrogen atom or an alkyl or substituted alkyl group or an alkoxy or substituted alkoxy group; n is a positive integer from 2 to 10 and alkyl contains from 1 to 6 carbon atoms. Among the useful alkyl radicals for R there may be mentioned —CH<sub>3</sub>, —C<sub>2</sub>H<sub>5</sub>, —CH(CH<sub>3</sub>)<sub>2</sub> and among the useful substituted alkyl radicals R there may be mentioned —CH<sub>2</sub>OH and —CH<sub>2</sub>Cl. Suitable specific alkoxy radicals for R include —OCH<sub>3</sub> and —OC<sub>2</sub>H<sub>5</sub>, —OCH(CH<sub>3</sub>)<sub>2</sub>. R, however, preferably is hydrogen or an unsubstituted alkyl or alkoxy radical of 1 to 3 carbon atoms.

It is important that the tertiary nitrogen atom and the sulfophenyl group in the above compounds be separated by at least two methylene (CH<sub>2</sub>) groups in order to obtain a high degree

2

of photographic development. The compounds where n is 3 to 6 and alkyl contains 1 to 4 carbon atoms are preferred. When n is greater than 10 the compounds still possess some developing properties but are less satisfactory than compounds covered by Formula I because the developer has a slow rate of diffusion into a colloid silver halide emulsion layer and it is more difficult to wash such compounds out of the colloid silver halide emulsion layers.

10 The compounds of Formula I may be prepared by the following series of chemical reactions: (a) preparation of an N-alkyl-N-(phenoxyalkyl)-aniline by reaction of an omega-halogen substituted alkyl phenylether containing the halogen and ether groups on the opposite ends of the straight chain alkylene radical with an N-alkylaniline, e. g., N-methylaniline, N-ethylaniline or N-butylaniline. This reaction is usually carried out under neutral to alkaline conditions; (b) preparation of N-alkyl-N-(omega-sulfophenyloxyalkyl) anilines by the reaction of the tertiary amine derivative obtained in step a with a sulfonating agent, e. g., hot concentrated sulfuric acid; (c) preparation of the corresponding p-nitroso-N-alkyl-N-(omega-sulfophenyloxyalkyl) aniline by reaction of the compound obtained in step b with nitrous acid; and (d) reduction of the nitroso compound obtained in step c, e. g., with iron or catalytically with hydrogen to the corresponding amine having the general Formula I.

When N-methyl, ethyl-m-toluidine, N-methyl, ethyl-m-anisidine, or similarly nuclear substituted N-alkyl anilines are used in place of N-alkyl aniline in the above syntheses one obtains the correspondingly substituted developers.

This invention will be further illustrated by the following examples. They exemplify suitable specific methods for the preparation of the compounds and illustrate their uses and properties but are not intended to limit the invention.

## EXAMPLE I

## p-AMINO-N-ETHYL-N-[OMEGA-(p-SULFOPHOXY)-PROPYL]ANILINE

## A. N-ethyl-N-(omega-phenoxypropyl) aniline

Omega-bromopropyl phenyl ether (215 grams, 0.5 mol) and N-ethylaniline (242 grams, 1 mol) were heated on a steam bath for 15 hours. The product was washed with a solution of 22 grams of sodium hydroxide in 300 milliliters of H<sub>2</sub>O followed by a water wash, and dried. Distillation gave 209 grams (92%) at 186-8° C./2 mm.; 55 n<sub>D</sub><sup>25</sup> = 1.5753.

**B. *N*-ethyl-*N*-[omega-(*p*-sulfophenoxy)propyl]-aniline**

*N*-ethyl-*N*-(omega-phenoxypropyl) aniline (51 grams) was added in a thin stream to 45 ml. of sulfuric acid in a stirred flask. The mixture was kept at 90° C. for 0.5 hour, then cooled and poured onto 75 grams of ice. The aqueous layer was removed from the syrup which separated and replaced with 75 milliliters of water. The product crystallized on standing. It was recrystallized from water; yield 32 grams, M. P. 222-4° C.

**C. *p*-Nitroso-*N*-ethyl-*N*-[omega-(*p*-sulfophenoxy)-propyl]aniline**

One hundred grams of *N*-ethyl-*N*-[omega-*p*-sulfophenoxy)propyl]aniline was dissolved in 90 milliliters of hydrochloric acid plus 35 milliliters of water. The solution was cooled to 0° C. and 20.4 grams of sodium nitrite in 40 milliliters of water was added with stirring at 0-5° C. After 3/4 hour of stirring, 250 milliliters of water was added, the mixture was seeded, and stirring was continued for 15 minutes. The nitroso compound was then filtered off and washed with water. Yield, 106 grams. It was only slightly soluble in hot water or alcohol.

Analysis Calculated for  $C_{17}H_{20}N_2O_5S$ : N, 7.69. Found: N, 7.57.

**D. *p*-Amino-*N*-ethyl-*N*-[omega-(*p*-sulfophenoxy)-propyl]aniline**

Ninety-one grams of the above nitroso compound was dissolved in 10 grams of NaOH plus 130 milliliters of water, charged into a shaker tube with 2 grams of palladium-on-charcoal catalyst and hydrogenated at 25-55° C. and 200-1000 lbs./sq. in. for one hour.

The product was treated with a little sodium hydrosulfite and a decolorizing charcoal and filtered. The pH of the solution was adjusted to 6 which caused the product to separate as a syrup. The water was separated and the syrup was rubbed with dioxane to cause it to crystallize. Yield, 86 grams (82%).

**EXAMPLE II**

**P-AMINO-*N*-ETHYL-*N*-[4-(*p*-SULFOPHENOXY)BUTYL]-ANILINE**

**A. 4-phenoxybutyl bromide**

In a 2-liter, 3-necked flask equipped with a stirrer, condenser and dropping funnel were placed 158 grams of 88% phenol, 402 grams of tetramethylenedibromide and 750 milliliters of water. The mixture was refluxed and during 0.5 hour 57 grams of sodium hydroxide in 190 milliliters of water was added. The mixture was refluxed five hours longer, after which it was cooled, the organic layer was separated, dried and distilled. A 50% yield (169 grams) of 4-phenoxybutyl bromide, boiling at 166-170° C./20 mm. was obtained.

**B. *N*-ethyl-*N*-(4-phenoxybutyl) aniline**

4-phenoxybutyl bromide (168 grams) and *N*-ethyl aniline (178 grams) were heated three hours at 125° C. The product was cooled and shaken with 32 grams of sodium hydroxide in 500 cc. of water. The amine was separated, dried and distilled and 81% yield (159 grams) boiling at 226-9° C./2 mm. was obtained;  $n_D^{25}=1.5709$ .

**C. *N*-ethyl-*N*-[4-(sulfophenoxy)butyl]aniline**

*N*-ethyl-*N*-(4-phenoxybutyl) aniline (159 grams) was run in a thin stream into 127 milliliters of sulfuric acid with cooling so that the temperature did not rise above 90° C. The solution was heated on a steam bath at 90-96° C. for 0.5 hour. The mixture was poured onto 200 grams of ice and the solution of the sulfonated products, which was completely soluble in sodium hydroxide solution, was used directly for nitrosation.

**D. *p*-Nitroso-*N*-ethyl-*N*-[4-(*p*-sulfophenoxy)-butyl]aniline**

The above solution was mixed with 75 milliliters of hydrochloric acid and stirred at 0-5° C. while 43 grams of sodium nitrite in 60 milliliters of water was added dropwise. Crystallization was started by scratching the product. After the mixture had stirred for one hour, the nitroso compound was filtered off and washed with water. The yield was 174 grams or 78%. The compound may be crystallized in small portions from water.

**E. *p*-Amino-*N*-ethyl-*N*-[4-(*p*-sulfophenoxy)-butyl]aniline**

Eighty-five grams of the above nitroso compound was dissolved in 120 milliliters of water containing 9 grams of sodium hydroxide and charged into a shaker tube with 2 grams of palladium-on-charcoal catalyst. Hydrogenation was carried out at 25-50° C. and 1500 lbs./sq. in. for one hour. The product was mixed with 50 milliliters of hydrochloric acid and the catalyst was filtered off with the aid of a silicous filtering aid. A small amount of sodium hydrosulfite was added to the filtrate and sodium hydroxide solution was added to a pH of about 6. A yield of 62.5 grams of the amino acid separated. The amino acid was recrystallized from water. The compound had water of crystallization which was gradually lost on heating in an oven, but it appears that the compound separates with two molecules of water.

Analysis calculated for  $C_{18}H_{24}N_2O_4S \cdot 2H_2O$ : N, 7.00. Found: N, 6.94, 6.84.

**EXAMPLE III**

**P-AMINO-*N*-ETHYL-*N*-[6-(*p*-SULFOPHENOXY)HEXYL]-ANILINE**

**A. 6-phenoxyhexyl bromide**

A stirred mixture of 300 grams of hexamethylene dibromide, 105 grams of 88% phenol and 500 milliliters of water was refluxed while 37.5 grams of sodium hydroxide in 125 milliliters of water was added during 0.5 hour. After five hours of reflux, the mixture was cooled and the organic layer was separated, dried and distilled. The yield of 6-phenoxyhexyl bromide, boiling at 176-186° C./9 mm., was 63 grams or 25%;  $n_D^{25}=1.5281$ .

**B. *N*-ethyl-*N*-(6-phenoxyhexyl) aniline**

6-phenoxyhexyl bromide (51.5 grams, 0.2 mol) and *N*-ethyl aniline (48.5 grams, 0.4 mol) were heated for 15 hours on a steam bath. The product was shaken with 10 grams of sodium hydroxide in 100 milliliters of water and the amine layer was separated, dried and distilled. The yield of *N*-ethyl-*N*-(6-phenoxyhexyl) aniline was 43.5 grams or 73%; B. P. 208-14°/1.5 mm.;  $n_D^{25}=1.5582$ .

C. *N*-ethyl-*N*-(6-(*p*-sulfophenoxy)hexyl)aniline

*N*-ethyl-*N*-(6-phenoxyhexyl) aniline (41 grams) was added to 33 milliliters of sulfuric acid with stirring. The temperature was kept at 90° C. during the addition and the mixture was then heated at 90-95° C. for 0.5 hour. The sulfonated product was cooled and poured onto 100 grams

types of compounds of this invention as compared with those of *p*-amino-*N,N*-diethyl aniline are set forth in the following table:

Table



|         | Block Speed |     |     |     |     | Gamma |      |      |      |      | Base+Fog |      |      |      |      |
|---------|-------------|-----|-----|-----|-----|-------|------|------|------|------|----------|------|------|------|------|
|         | CD-1        | n=2 | n=3 | n=4 | n=6 | CD-1  | n=2  | n=3  | n=4  | n=6  | CD-1     | n=2  | n=3  | n=4  | n=6  |
| Cyan    | 5.0         | 3.1 | 4.6 | 4.7 | 5.0 | 3.70  | 2.55 | 4.23 | 4.24 | 4.05 | 0.13     | 0.11 | 0.13 | 0.13 | 0.14 |
| Magenta | 6.7         | 4.2 | 6.2 | 5.7 | 7.0 | 2.14  | 1.25 | 2.51 | 1.73 | 1.71 | 0.20     | 0.15 | 0.19 | 0.12 | 0.16 |
| Yellow  | 6.0         | 3.0 | 4.6 | 4.7 | 5.4 | 1.93  | 0.40 | 1.42 | 1.82 | 1.58 | 0.09     | 0.08 | 0.08 | 0.08 | 0.09 |

## MULTILAYER COATINGS

|         |     |     |     |     |     |      |      |      |      |      |      |      |      |      |      |
|---------|-----|-----|-----|-----|-----|------|------|------|------|------|------|------|------|------|------|
| Cyan    | 5.2 | 3.7 | 4.8 | 4.7 | 5.3 | 3.36 | 2.57 | 3.72 | 3.83 | 3.29 | 0.12 | 0.11 | 0.15 | 0.10 | 0.32 |
| Magenta | 4.5 | 1.6 | 3.3 | 3.5 | 4.3 | 2.48 | 0.62 | 2.27 | 2.69 | 2.34 | 0.11 | 0.09 | 0.12 | 0.14 | 0.28 |
| Yellow  | 4.6 | 1.8 | 3.5 | 3.9 | 3.6 | 1.44 | 0.32 | 1.64 | 1.34 | 1.00 | 0.14 | 0.09 | 0.09 | 0.14 | 0.26 |

CD-1 = *p*-Amino-*N,N*-diethyl aniline.

of ice. This solution was used directly for nitrosation after 50 milliliters of water and 120 milliliters of hydrochloric acid were added.

D. *p*-Nitroso-*N*-ethyl-*N*-(6-(*p*-sulfophenoxy)-hexyl)aniline

To the above solution was added with stirring 10 grams of sodium nitrite in 15 milliliters of water at 0-5° C. The mixture was stirred for one hour, 400 milliliters of water was added, and the inside of the flask was scratched to induce crystallization. After two additional hours of stirring, the nitroso compound was filtered off and washed with water. The yield was 39 grams or 70%. The compound was recrystallized from water.

E. *p*-Amino-*N*-ethyl-*N*-(6-(sulfophenoxy)-hexyl)aniline

Thirty grams of the above nitroso compound was dissolved in a solution of 3 grams of sodium hydroxide in 100 milliliters of water and charged into a shaker tube with 2 grams of palladium-on-charcoal catalyst and hydrogenated at 50-60° C. and 1500 lbs./sq. in. for 1.5 hours. The product was filtered and one equivalent of hydrochloric acid was added to precipitate the amino acid as a syrup. The syrup was rubbed with dioxane to cause it to crystallize. The yield was 21 grams. The product was recrystallized from water.

Analysis calculated for  $\text{C}_{10}\text{H}_{22}\text{N}_2\text{O}_4\text{S} \cdot 2\text{H}_2\text{O}$ : N, 6.56. Found: N, 6.64, 6.69.

## EXAMPLE IV

p-AMINO-*N*-ETHYL-*N*[(BETA-(*p*-SULFOPHOXY)-ETHYL)ANILINE

When the general procedure of Example I was repeated except that beta-bromoethyl phenyl ether was employed in place of the omega-bromo-propyl phenyl ether there was obtained upon condensation with aniline, *N*-ethyl-*N*-(beta-phenoxyethyl)aniline, B. P. 154-156°/3 mm.;  $n_{D}^{25}=1.5860$ .

Treatment with sulfuric acid gave *N*-ethyl-*N*-(beta-(*p*-sulfophenoxy)ethyl)aniline. Treatment of the latter under acid conditions with sodium nitrite gave *p*-nitroso-*N*-ethyl-*N*-(beta-(*p*-sulfophenoxy)ethyl)aniline, which upon reduction gave the corresponding amino compound. The hydrochloride had the following analysis:

Calculated for  $\text{C}_{10}\text{H}_{22}\text{N}_2\text{O}_4\text{S}$ : N, 7.53; S, 8.60. Found: N, 7.58; S, 9.09.

The photographic developing properties of the

50  
55  
60  
65  
70  
75  
80  
85  
90  
95  
100

types of compounds of this invention as compared with those of *p*-amino-*N,N*-diethyl aniline are set forth in the following table:

Sensitometric  
 Data for  $\text{H}_2\text{N}-\text{C}_6\text{H}_4-\text{N}(\text{CH}_3)_2-\text{O}-\text{C}_6\text{H}_4-\text{SO}_3\text{H}$   
 MONOLAYER COATINGS

|         | Block Speed |     |     |     |     | Gamma |      |      |      |      | Base+Fog |      |      |      |      |
|---------|-------------|-----|-----|-----|-----|-------|------|------|------|------|----------|------|------|------|------|
|         | CD-1        | n=2 | n=3 | n=4 | n=6 | CD-1  | n=2  | n=3  | n=4  | n=6  | CD-1     | n=2  | n=3  | n=4  | n=6  |
| Cyan    | 5.0         | 3.1 | 4.6 | 4.7 | 5.0 | 3.70  | 2.55 | 4.23 | 4.24 | 4.05 | 0.13     | 0.11 | 0.13 | 0.13 | 0.14 |
| Magenta | 6.7         | 4.2 | 6.2 | 5.7 | 7.0 | 2.14  | 1.25 | 2.51 | 1.73 | 1.71 | 0.20     | 0.15 | 0.19 | 0.12 | 0.16 |
| Yellow  | 6.0         | 3.0 | 4.6 | 4.7 | 5.4 | 1.93  | 0.40 | 1.42 | 1.82 | 1.58 | 0.09     | 0.08 | 0.08 | 0.08 | 0.09 |

MULTILAYER COATINGS

|         |     |     |     |     |     |      |      |      |      |      |      |      |      |      |      |
|---------|-----|-----|-----|-----|-----|------|------|------|------|------|------|------|------|------|------|
| Cyan    | 5.2 | 3.7 | 4.8 | 4.7 | 5.3 | 3.36 | 2.57 | 3.72 | 3.83 | 3.29 | 0.12 | 0.11 | 0.15 | 0.10 | 0.32 |
| Magenta | 4.5 | 1.6 | 3.3 | 3.5 | 4.3 | 2.48 | 0.62 | 2.27 | 2.69 | 2.34 | 0.11 | 0.09 | 0.12 | 0.14 | 0.28 |
| Yellow  | 4.6 | 1.8 | 3.5 | 3.9 | 3.6 | 1.44 | 0.32 | 1.64 | 1.34 | 1.00 | 0.14 | 0.09 | 0.09 | 0.14 | 0.26 |

CD-1 = *p*-Amino-*N,N*-diethyl aniline.

of ice. This solution was used directly for nitrosation after 50 milliliters of water and 120 milliliters of hydrochloric acid were added.

*p*-Nitroso-*N*-ethyl-*N*-(6-(*p*-sulfophenoxy)-hexyl)aniline

To the above solution was added with stirring 10 grams of sodium nitrite in 15 milliliters of water at 0-5° C. The mixture was stirred for one hour, 400 milliliters of water was added, and the inside of the flask was scratched to induce crystallization. After two additional hours of stirring, the nitroso compound was filtered off and washed with water. The yield was 39 grams or 70%. The compound was recrystallized from water.

*p*-Amino-*N*-ethyl-*N*-(6-(sulfophenoxy)-hexyl)aniline

Thirty grams of the above nitroso compound was dissolved in a solution of 3 grams of sodium hydroxide in 100 milliliters of water and charged into a shaker tube with 2 grams of palladium-on-charcoal catalyst and hydrogenated at 50-60° C. and 1500 lbs./sq. in. for 1.5 hours. The product was filtered and one equivalent of hydrochloric acid was added to precipitate the amino acid as a syrup. The syrup was rubbed with dioxane to cause it to crystallize. The yield was 21 grams. The product was recrystallized from water.

Analysis calculated for  $\text{C}_{10}\text{H}_{22}\text{N}_2\text{O}_4\text{S} \cdot 2\text{H}_2\text{O}$ : N, 6.56. Found: N, 6.64, 6.69.

**EXAMPLE IV**

**p-AMINO-*N*-ETHYL-*N*[(BETA-(*p*-SULFOPHOXY)-ETHYL)ANILINE**

When the general procedure of Example I was repeated except that beta-bromoethyl phenyl ether was employed in place of the omega-bromo-propyl phenyl ether there was obtained upon condensation with aniline, *N*-ethyl-*N*-(beta-phenoxyethyl)aniline, B. P. 154-156°/3 mm.;  $n_{D}^{25}=1.5860$ .

Treatment with sulfuric acid gave *N*-ethyl-*N*-(beta-(*p*-sulfophenoxy)ethyl)aniline. Treatment of the latter under acid conditions with sodium nitrite gave *p*-nitroso-*N*-ethyl-*N*-(beta-(*p*-sulfophenoxy)ethyl)aniline, which upon reduction gave the corresponding amino compound. The hydrochloride had the following analysis:

Calculated for  $\text{C}_{10}\text{H}_{22}\text{N}_2\text{O}_4\text{S}$ : N, 7.53; S, 8.60. Found: N, 7.58; S, 9.09.

The photographic developing properties of the

types of compounds of this invention as compared with those of *p*-amino-*N,N*-diethyl aniline are set forth in the following table:

Sensitometric  
 Data for  $\text{H}_2\text{N}-\text{C}_6\text{H}_4-\text{N}(\text{CH}_3)_2-\text{O}-\text{C}_6\text{H}_4-\text{SO}_3\text{H}$   
 MONOLAYER COATINGS

|         | Block Speed |     |     |     |     | Gamma |      |      |      |      | Base+Fog |      |      |      |      |
|---------|-------------|-----|-----|-----|-----|-------|------|------|------|------|----------|------|------|------|------|
|         | CD-1        | n=2 | n=3 | n=4 | n=6 | CD-1  | n=2  | n=3  | n=4  | n=6  | CD-1     | n=2  | n=3  | n=4  | n=6  |
| Cyan    | 5.0         | 3.1 | 4.6 | 4.7 | 5.0 | 3.70  | 2.55 | 4.23 | 4.24 | 4.05 | 0.13     | 0.11 | 0.13 | 0.13 | 0.14 |
| Magenta | 6.7         | 4.2 | 6.2 | 5.7 | 7.0 | 2.14  | 1.25 | 2.51 | 1.73 | 1.71 | 0.20     | 0.15 | 0.19 | 0.12 | 0.16 |
| Yellow  | 6.0         | 3.0 | 4.6 | 4.7 | 5.4 | 1.93  | 0.40 | 1.42 | 1.82 | 1.58 | 0.09     | 0.08 | 0.08 | 0.08 | 0.09 |

MULTILAYER COATINGS

|         |     |     |     |     |     |      |      |      |      |      |      |      |      |      |      |
|---------|-----|-----|-----|-----|-----|------|------|------|------|------|------|------|------|------|------|
| Cyan    | 5.2 | 3.7 | 4.8 | 4.7 | 5.3 | 3.36 | 2.57 | 3.72 | 3.83 | 3.29 | 0.12 | 0.11 | 0.15 | 0.10 | 0.32 |
| Magenta | 4.5 | 1.6 | 3.3 | 3.5 | 4.3 | 2.48 | 0.62 | 2.27 | 2.69 | 2.34 | 0.11 | 0.09 | 0.12 | 0.14 | 0.28 |
| Yellow  | 4.6 | 1.8 | 3.5 | 3.9 | 3.6 | 1.44 | 0.32 | 1.64 | 1.34 | 1.00 | 0.14 | 0.09 | 0.09 | 0.14 | 0.26 |

CD-1 = *p*-Amino-*N,N*-diethyl aniline.

of ice. This solution was used directly for nitrosation after 50 milliliters of water and 120 milliliters of hydrochloric acid were added.

*p*-Nitroso-*N*-ethyl-*N*-(6-(*p*-sulfophenoxy)-hexyl)aniline

To the above solution was added with stirring 10 grams of sodium nitrite in 15 milliliters of water at 0-5° C. The mixture was stirred for one hour, 400 milliliters of water was added, and the inside of the flask was scratched to induce crystallization. After two additional hours of stirring, the nitroso compound was filtered off and washed with water. The yield was 39 grams or 70%. The compound was recrystallized from water.

*p*-Amino-*N*-ethyl-*N*-(6-(sulfophenoxy)-hexyl)aniline

Thirty grams of the above nitroso compound was dissolved in a solution of 3 grams of sodium hydroxide in 100 milliliters of water and charged into a shaker tube with 2 grams of palladium-on-charcoal catalyst and hydrogenated at 50-60° C. and 1500 lbs./sq. in. for 1.5 hours. The product was filtered and one equivalent of hydrochloric acid was added to precipitate the amino acid as a syrup. The syrup was rubbed with dioxane to cause it to crystallize. The yield was 21 grams. The product was recrystallized from water.

Analysis calculated for  $\text{C}_{10}\text{H}_{22}\text{N}_2\text{O}_4\text{S} \cdot 2\text{H}_2\text{O}$ : N, 6.56. Found: N, 6.64, 6.69.

**EXAMPLE IV**

**p-AMINO-*N*-ETHYL-*N*[(BETA-(*p*-SULFOPHOXY)-ETHYL)ANILINE**

When the general procedure of Example I was repeated except that beta-bromoethyl phenyl ether was employed in place of the omega-bromo-propyl phenyl ether there was obtained upon condensation with aniline, *N*-ethyl-*N*-(beta-phenoxyethyl)aniline, B. P. 154-156°/3 mm.;  $n_{D}^{25}=1.5860$ .

Treatment with sulfuric acid gave *N*-ethyl-*N*-(beta-(*p*-sulfophenoxy)ethyl)aniline. Treatment of the latter under acid conditions with sodium nitrite gave *p*-nitroso-*N*-ethyl-*N*-(beta-(*p*-sulfophenoxy)ethyl)aniline, which upon reduction gave the corresponding amino compound. The hydrochloride had the following analysis:

Calculated for  $\text{C}_{10}\text{H}_{22}\text{N}_2\text{O}_4\text{S}$ : N, 7.53; S, 8.60. Found: N, 7.58; S, 9.09.

The photographic developing properties of the

As many widely different embodiments of this invention can be made without departing from the spirit and scope thereof, it is to be understood that the invention is not to be limited except as defined by the claims.

What is claimed is:

1. The chemical compounds of the general formula:



where R is a member taken from the group consisting of hydrogen, alkyl radicals of 1 to 3 carbon atoms and alkoxy radicals of 1 to 3 carbon atoms, alkyl contains 1 to 6 carbon atoms and n is a cardinal number from 2 to 6 inclusive.

2. p - Amino - N-ethyl-N-[omega-(p-sulfophenoxy)propyl]aniline.

3. p - Amino-N-ethyl-N-[4-(p-sulfophenoxy)-butyl]aniline.

4. p - Amino-N-ethyl-N-[6-(p-sulfophenoxy)-hexyl]aniline.

ELMORE LOUIS MARTIN.

#### REFERENCES CITED

10 The following references are of record in the file of this patent:

#### UNITED STATES PATENTS

| Number    | Name            | Date          |
|-----------|-----------------|---------------|
| 2,163,166 | Wilmanns et al. | June 20, 1939 |
| 2,241,769 | Dickey et al.   | May 13, 1941  |